

317,388

## UNITED STATES PATENT OFFICE.

CHARLES S. LOCKWOOD, OF ALBANY, NEW YORK, AND JOHN W. HYATT,  
OF NEWARK, NEW JERSEY, ASSIGNEES TO THE BONSILATE COMPANY,  
(LIMITED,) OF ALBANY, N. Y.

## PROCESS OF TREATING SILICATE OF SODA IN COMBINATION WITH ZINC OXIDE, &amp;c.

SPECIFICATION forming part of Letters Patent No. 317,388, dated May 5, 1885.

Application filed August 13, 1884. (No specimens.)

18-47.5

*To all whom it may concern:*

Be it known that we, CHARLES S. LOCKWOOD, a citizen of the United States, and a resident of Albany, in the county of Albany and State of New York, and JOHN W. HYATT, a citizen of the United States, residing at Newark, Essex county, New Jersey, have invented a certain new and useful Improved Process of Treating Silicate of Soda in combination with Zinc Oxide and the Composition Produced by such Process, of which the following is a specification.

The invention has relation to an improved process of treating silicate of soda in combination with zinc oxide and to the composition produced by such process, as hereinafter set forth. We take silicate of soda, which is made into a solution, a sufficient quantity of water being added to enable a thorough filtration.

This solution we reduce to such an extent that at a temperature of 60° it has a specific gravity of about 26° Baumé. Of the solution of silicate of soda in the condition just stated we take, say, eight pounds, to which we add, say,

25 two pounds of white zinc oxide and mix the two as effectually as possible. We then place the mixture, preferably, on a water bath and evaporate it slowly until a sufficient part of the water has been removed to allow the ma-

30 terial to be comminuted. Before the comminution is attempted the compound will be allowed to cool, and will then be ground to a fine powder by means of a mill of any convenient kind, or reduced in any other way. It is

35 essential that great care be taken not to carry the evaporation too far. To ascertain whether the powder is in a proper condition to be subjected to the action of the mold, we have been accustomed to press it upon a

40 heated surface of polished metal. If it is in such a condition that it will not adhere to the metal surface when subjected to the degree of heat and pressure required to weld it, (say a temperature of about 300° Fahrenheit and a

45 pressure of, say, eight thousand pounds to the square inch,) the proper degree of desiccation will have been reached. The material, having been brought to a condition in which it is

ready to be subjected to heat and pressure, is introduced into molds of ordinary construction and pressed to form the desired article. The dies employed are of usual construction. They will be heated to a temperature of, say, 250° to 350° Farhenheit, or thereabout, and the material will be subjected to a pressure of 55 about, say, eight thousand pounds to the square inch, more or less, according to the character of the article, the heat and pressure being continued until a complete consolidation of the contents of the mold has been effected.

One of the chief difficulties connected with the utilization of alkaline silicates in the production of articles of commerce has been that after the article is completed it attracts moisture and has a tendency to effloresce to such an extent as to destroy its value. To correct these difficulties is one of the principal objects of our process, and it is accomplished by the use of a bath of ammoniacal salts, in which the 70 material is introduced after it is subjected to the action of the molds.

In practice we prefer to immerse the completed article in the bath after it has been moulded and polished.

Having proceeded in the formation of the article, as hereinbefore described, it is polished in any convenient way and then introduced into a bath consisting of, say, two parts of water to one part of chloride of ammonium, in 80 which it is permitted to remain from, say, ten to fifteen hours, or until a test shows that there is no further alkaline reaction. Any of the ammoniacal salts may be made use of, and the strength of the bath will be varied according 85 to circumstances.

It is not to be understood that we limit our claim to the exact proportion of silicate and zinc oxide described, as they may be varied to some extent, or that we contemplate the 90 employment of a bath of any particular strength, or that we limit our claim to the bath to the treatment of the particular compound we have described.

What we claim as our invention, and desire to secure by Letters Patent, is—

1. The within-described process of forming articles of silicate of soda and oxide of zinc, which consists in, first, forming an aqueous solution of the silicate of soda with an admixture of zinc oxide in the proportion of about four parts of silicate (26° Baumé) to one part of zinc oxide; second, desiccating and comminuting the compound, and, third, subjecting the desiccated powder to pressure in heated molds, and, fourth, treating the article in an ammoniacal bath, substantially as set forth.
2. The use of an ammoniacal bath for the purpose of correcting the tendency of an alkaline silicate to attract moisture and to effloresce, substantially as set forth.
3. The within-described process of forming articles of silicate of soda and oxide of zinc, which consists in, first, forming an aqueous solution of the silicate of soda with an admixture of zinc oxide in the proportion of about four parts of silicate (26° Baumé) to one part of zinc oxide, and, second, desiccating the compound, comminuting it, and subjecting it to treatment in an ammoniacal bath, substantially as set forth.

4. A composition consisting, essentially, of silicate of soda and zinc oxide combined, comminuted and partly dehydrated, substantially as set forth.

5. An article consisting of an alkaline silicate and white zinc oxide, combined in the proportions and united by heat and pressure substantially as set forth.

Signed at Albany, in the county of Albany and State of New York, this 2d day of August, 35 A. D. 1884.

CHAS. S. LOCKWOOD.

Witnesses:

ROBERT C. PRUYN,  
E. A. GROESBECK.

Signed at Newark, in the county of Essex and State of New Jersey, this 9th day of August, A. D. 1884.

JOHN W. HYATT.

Witnesses:

ABRAHAM MANNERS,  
CHAS. C. GILL.